

June 27, 1972

D. D. PETERSON

3,673,017

PARTICLE TRACK ETCHING METHOD

Filed July 9, 1970

FIG. 1



FIG. 2



FIG. 3



FIG. 4



INVENTOR:

DAVID D. PETERSON,

by *Paul C. Frank*  
HIS ATTORNEY

1

3,673,017

## PARTICLE TRACK ETCHING METHOD

David D. Peterson, Bristol, England, assignor to  
General Electric Company

Filed July 9, 1970, Ser. No. 53,495  
Int. Cl. B44c 1/22; C23f 1/00

U.S. Cl. 156—7

5 Claims

### ABSTRACT OF THE DISCLOSURE

A new particle track etching method is disclosed where-  
in a smoother and more uniform track profile is obtained  
by controlling the chemical concentrations of the reagents  
and products so that the etching occurs at a uniform rate.  
Specifically, the etchant is maintained saturated with etch  
products throughout the entire etching procedure.

This invention relates to particle track etching methods  
and in particular to an improved method whereby the  
bore made by the etchant along the path of the particle  
has a uniform profile as opposed to an irregular profile  
obtained by present methods.

As is now well known, tracks left by atomic particles  
in solids can be enlarged for study by the use of an etchant  
solution. The enlarged bores made by the etchant solution,  
while suitable for studies relative to such things as the  
track length and direction, are not as suitable for such  
uses as filter elements having ultra-small holes as those of  
the present invention. This is because presently used etch-  
ants cause the hole to have a non-uniform profile.

In view of the above, it is therefore an object of the  
present invention to provide a particle track etching  
method wherein the bore made by the etchant has a  
uniform profile.

The foregoing object is achieved wherein the etchant  
material, from the start of the etchant process to the  
completion of that process, is a saturated solution; i.e.,  
saturated with the etch product. It has been found that  
as the etch product concentration is increased there is  
an abrupt change in the etching rate at the solubility limit  
of the etch products. By controlling the etching process  
so that it takes place at the maximum rate over the entire  
surface of the material being etched, a uniform profile is  
obtained along the particle track.

A more complete understanding of the present invention  
may be obtained by considering the following detailed  
description in conjunction with the attached drawing in  
which:

FIG. 1 illustrates the general etching process.

FIG. 2 is a plan view of a comparison of the etching  
process according to the present invention and that of  
the prior art.

FIG. 3 is a side view of a comparison of the etching  
process according to the present invention and that of  
the prior art.

FIG. 4 illustrates curves showing bulk etching rate as  
a function of etch product concentration.

Referring to FIG. 1 there is shown a block of material  
10 containing a particle track 11. The material 10 may  
comprise any suitable dielectric material such as a plastic  
film which, for example, may be Lexan polycarbonate  
film. As a charged particle passes through film 10, it  
leaves a track of damage 11.

Upon being subjected to an etching solution, the surface  
of the film 10 is etched away together with region along  
the track 11. The rate at which the surface of the film 10  
is worn away is known as the general etching rate. The  
rate at which the track is etched away is called the track  
etching rate. To obtain a track upon etching, the track

2

etching rate must be larger than the general etching rate  
and the ratio of these two determines the shape of the  
bore left by the etching solution. The configuration of  
film 10 after being subjected to the etching solution is  
illustrated by dashed lines 12 and 13. The thickness of  
the film 10 has been reduced to the point indicated by  
line 13 and is determined by the general etching rate.  
The enlarged track portion 12, which may be conical in  
shape, has its height determined by the track etching rate.  
The profile of the bore 12 is generally rather irregular  
when etchants of the prior art are used. It has been dis-  
covered that upon saturation of the etchant solution with  
etch products, the rate of etching abruptly increases to a  
maximum and remains at the level for as long as the etch-  
ing solution remains saturated. Utilizing this method,  
much of the irregularity of profile can be alleviated.

A comparison of the method of the prior art and that  
of the present invention is illustrated in FIGS. 2 and 3.  
As shown in FIGS. 2 and 3, the bore 15 resulting from  
the etchings of the prior art has an irregular profile 14.

In accordance with the present invention in which the  
etchant solution is presaturated with etch products,  
the resulting etching takes place at a maximum and a  
uniform rate resulting in a bore 17 of uniform profile 16.

FIG. 4 illustrates a set of curves showing the bulk  
etching rate as a function of etch product concentration  
for two different etchant temperatures, namely, 40° C.  
and 55° C. An example of an etchant that may be used  
for Lexan is a 6.25 N aqueous sodium hydroxide solution  
containing a 0.05 percent Benax 2A1 surfactant or wetting  
agent. Benax 2A1 is made by Dow Chemical Company.  
As can be seen from FIG. 3, an etching solution at 40° C.  
has a bulk etching rate of about 0.08 micron per hour  
until the etch product solubility limit is reached, where-  
upon the bulk etching rate abruptly changes to about 0.17  
micron per hour. Similarly, the bulk etching rate with  
a 55° C. etchant gradually increases until the etch product  
solubility limit is reached whereupon it can abruptly in-  
creases to a stable value. Thus, by utilizing an etchant  
that is saturated with etch products, a smooth bore along  
the particle track is obtained.

Having thus described the invention, it will be apparent  
to those skilled in the art that modifications may be made  
within the scope of the present invention. For example,  
the method of the present invention may be used in other  
areas in which materials are etched, as in the semiconductor  
fabrication art.

What I claim as new and desire to secure by Letters  
Patent of the United States is:

1. An etching method for etching a material with an  
etching solution producing etch products comprising the  
steps of:  
presaturating said etching solution with said etch  
products,  
subjecting said material to be etched to said presaturated  
etching solution, and  
maintaining said etching solution saturated with said  
etch products during the etching of said material.
2. A method for etching a material containing particle  
tracks with an etching solution producing etch products  
comprising the steps of:  
presaturating said etching solution with said etch  
products,  
subjecting said material containing particle tracks to  
said presaturated etching solution, and  
maintaining said etching solution saturated with said  
etch products during the etching of said material.
3. A process as set forth in claim 2 wherein said etching  
solution comprises an aqueous hydroxide solution and a  
surfactant, and said material containing particle tracks  
comprises a polycarbonate film.

4. A particle track etching process comprising the steps of:

subjecting a material containing particle tracks to an etching solution, presaturated with etch products, and maintaining the rate of etching of said material at a predetermined level, whereby the etching of the material will produce a uniformly dimensioned etched particle track.

5. A particle track etching process as set forth in claim 4 wherein said predetermined level is the maximum etching rate.

4 References Cited

UNITED STATES PATENTS

|           |         |                  |          |
|-----------|---------|------------------|----------|
| 3,373,683 | 3/1968  | Alter            | 250—83 X |
| 3,415,993 | 12/1968 | Fleischer et al. | 156—2 X  |
| 3,418,472 | 12/1968 | Evans            | 250—83   |

ROBERT F. BURNETT, Primary Examiner

R. L. MAY, Assistant Examiner

U.S. Cl. X.R.

250—83 C D